

## UNITED STATES PATENT OFFICE

2,016,737

PROCESS FOR THE MANUFACTURE OF AZO  
DYESTUFFSGérald Bonhôte, Basel, Switzerland, assignor to  
Society of Chemical Industry in Basle, Basel,  
SwitzerlandNo Drawing. Application March 7, 1935, Serial  
No. 9,900. In Switzerland March 22, 1934

4 Claims. (Cl. 260—95)

In Patent No. 1,871,946 there is described a series of dyestuffs which dye violet tints and are obtained by the coupling of an arylide of 2,3-hydroxynaphthoic acid with a diazo-compound of the general formula



in which R is an aromatic nucleus of the benzene series and both X's are alkoxy-groups.

In the further working of this invention it has been observed that while these diazo-components in which both X's stand for  $OCH_3$  couple easily, considerable difficulty attends the coupling in the case of diazo-components in which both X's stand for  $OC_2H_5$ -groups. If the coupling is conducted in a medium acid with acetic acid the dyeings produced by the dyestuffs are weak and unsightly; if the coupling is conducted in neutral or feebly alkaline medium, such as a medium alkaline with bicarbonate of soda, the dyeings especially these on yarn, are stripy and, in consequence of the decomposition of the diazo-compound the dye-bath becomes turbid.

This invention relates to a process of making dyestuffs in substance or on the fibre of the constitution in question which yield unobjectionable dyeings by conducting the coupling in a liquid which, by suitable addition, retains a pH-value which is always markedly below 1 that is to say does not exceed 6.5 but does not substantially fall below 4.8. Thus the invention comprises the addition to the coupling solution of a buffer agent such as a mono-alkali salt of phosphoric acid and products of similar action whose pH-value lies about 5. Such buffer agents are for example the alkali salts of citric acid, mixtures of mono-potassium salts of phthalic acid with sodium hydroxide, mixtures of mono-alkali salts of maleic acid with dialkali salts of the same acid. This expedient leads to valuable results not only in the case of arylides of 2,3-hydroxynaphthoic acid but also in the case of other suitable hydroxy-carboxylic acids, for instance the arylides of 2,3-hydroxyanthracene-carboxylic acid. The addition of the buffer agent is also of value in the case of those diazo-components in which both

X's stand for  $OCH_3$ . As already stated the coupling of these diazo-components occurs more easily than that of the corresponding ethyl bodies; by use of the buffer substance the dyestuff obtained produces dyeings which are of equally good yield as those obtained with dyestuffs produced in neutral or feebly alkaline media; however, the baths remain completely clear when the buffer agent is used.

The following examples illustrate the invention:

## Example 1

Cotton yarn is impregnated with a solution containing per litre 5 grams of 2,3-hydroxy-naphthoic acid-1'-naphthalide, 14 cc. of caustic soda lye of 34° Bé., 10 cc. of Turkey red oil and 7 cc. of formaldehyde solution of 40 per cent. strength, then well wrung out and developed in a diazo-solution containing per litre the diazo-compound from 2 grams of 4-(4'-methyl)-phenoxyacetyl-amino-2,5-diethoxy-1-aminobenzene and 8 grams of primary potassium phosphate. There is obtained a pure blue tint.

The procedure is similar when other diazo-bases are used, for instance 4-phenoxy-acetylamino-2,5-diethoxy-1-aminobenzene, 4-(4'-chloro)-phenoxy-acetylamino-2,5-diethoxy-1-aminobenzene, 4-(2'- or 3' methyl)-phenoxy-acetylamino-2,5-diethoxy-1-aminobenzene and 30 when other arylides of 2,3-hydroxynaphthoic acid are used, for example the anilide, the metoluidide, the meta-chloraniline of 2,3-hydroxynaphthoic acid.

## Example 2

Cotton yarn is impregnated with a solution containing per litre 4 grams of 2,3-hydroxy-naphthoic acid-4'-ethoxyanilide, 8 cc. of caustic soda lye of 34° Bé., 10 cc. of Turkey red oil and 5 cc. of formaldehyde solution of 40 per cent. strength, well wrung out and developed in a diazo-solution containing the diazo-compound from 2 grams of 4-(4'-methyl)-phenoxyacetylamino-2,5-dimethoxy-1-aminobenzene and 10 45 grams of primary sodium phosphate per litre. There is produced a pure violet tint and the coupling bath remains completely clear.

Like results are obtained in printing or in dyeing piece goods. Other arylides of other acids 50

may be used, for example the arylides of 2,3-hydroxyanthracene-carboxylic acid.

What I claim is:—

1. A manufacture of dyestuffs in substance or on the fibre consisting in coupling a diazo-compound of the general formula



in which R is an aromatic nucleus of the benzene series and both X's stand for alkoxy-groups, with an arylide of an ortho-hydroxy carboxylic acid, capable of coupling in ortho-position to the OH-group, in a medium whose pH-value does not exceed 6.5 and does not fall substantially below 5.

2. A manufacture of dyestuffs in substance or on the fibre consisting in coupling a diazo-compound of the general formula



in which R is an aromatic nucleus of the benzene series and both X's stand for alkoxy-groups, with an arylide of the 2,3-hydroxynaphthoic acid, in a medium whose pH-value does not ex-

ceed 6.5 and does not fall substantially below 5

3. A manufacture of dyestuffs in substance or on the fibre consisting in coupling a diazo-compound of the general formula



in which R is an aromatic nucleus of the benzene series and both X's stand for alkoxy-groups, with an arylide of the 2,3-hydroxynaphthoic acid in a medium buffered by addition of a mono-alkali metal salt of phosphoric acid. 15

4. A manufacture of dystuffs in substance or on the fibre consisting in coupling a diazo-compound of the general formula 15



in which R is an aromatic nucleus of the benzene series, with an arylide of the 2,3-hydroxynaphthoic acid, in a medium buffered by addition of a mono-alkali metal salt of phosphoric acid. 25

GÉRALD BONHÔTE. 30